

## UNITED STATES PATENT OFFICE

2,171,427

## WRAPPING MATERIAL

John Eggert, Leipzig, and Bruno Wendt, Dessau, Germany, assignors to I. G. Farbenindustrie Aktiengesellschaft, Frankfort - on - the - Main, Germany

No Drawing. Application May 19, 1937, Serial No. 143,493. In Germany March 20, 1937

8 Claims. (Cl. 91—68)

Our present invention relates to a wrapping material and more particularly to an improved wrapping material for goods sensitive to light and air.

5 One of its objects is to provide a process of producing such wrapping material. Further objects will be seen from the detailed specification following hereafter.

It is known that the access of air and the 10 action of light, particularly ultra-violet light, damage the durability of goods of various kinds. For this reason, in packing goods such as articles of food, books, textile goods and the like, there are used protective casings of paper, regenerated 15 cellulose, superficially saponified cellulose acetate, gelatin and the like, which by saturation with a solution of aesculine or quinine sulfate have been made impermeable to ultra-violet light without detracting considerably from the transparency of 20 the casing to non-injurious light so that the packed goods can be seen through the packing. Such packings, which are particularly suitable for use in show windows, automatic machines and the like, have, however, the disadvantage that the substance which absorbs the ultra-violet light 25 is easily removed from the packing by moisture, so that the protective casing loses its power of absorbing ultra-violet light under action of moisture and the packed goods are liable to be contaminated with the substance that absorbs the 30 ultra-violet light when they contain moisture, for example foodstuffs.

This disadvantage is avoided or minimized 35 according to the present invention by using, as the substance that absorbs the ultra-violet light and is to be incorporated with the packing material, 1, 3, 5-triazine derivative. Among the

derivatives of 1, 3, 5-triazine there is a large number of bodies which, when incorporated with paper or regenerated cellulose or the like, lends sheets made with this material the property of absorbing ultra-violet light without essentially coloring the sheet. The triazine derivative becomes so intimately united with the paper fiber or other sheet material that on treatment with water or other usual solvent it is not removed from the material. Thus sheets containing 1, 3, 5-triazine derivatives are unobjectionable packings for goods which contain moisture, for example food-stuffs.

The following substances may be named as suitable for use as additions to transparent pack- 15 ing materials for the purpose in question:

1. N-[2, 4-dihydroxy-1, 3, 5-triazyl-(6)]-dehy-  
drothio-toluidine sulfonic acid:



2. Bis-[2, 4-dihydroxy-1, 3, 5-triazyl-(6)]-  
N,N'-benzidine disulfonic acid:



3. Bis-[2-hydroxy-4-diethylamino-1, 3, 5-tri-  
azyl-(6)]-N,N'-benzidine disulfonic acid:



4. Bis-[2-hydroxy-4-phenylamino-1, 3, 5-tri-  
azyl-(6)]-N,N'-benzidine disulfonic acid:



5. Bis-[2-(phenylamino)-4-(para-sulfophenylamino)-1, 3, 5-triazyl-(6)-N, N'-benzidine di-sulfonic acid;



6. 4, 4'-bis-[4-(2, 4-dihydroxy-1, 3, 5-triazyl-(6-amino)-benzamino]-diphenyl-disulfonic acid-(3, 3'):



30 7. Bis-[2-hydroxy-4 - phenylamino - 1,3,5 - tri-  
azyl-(6) ]-dianisidine-disulfonic acid:



### 8. 4,4'-bis-[2,4-dihydroxy-1,3,5-triazyl-(6)-amino]-diphenyl-dicarboxylic acid-(2,2'):



9. Bis-[2,4-dihydroxy-1,3,5-triazyl-(6)]-benzidine sulfone disulfonic acid:



65 10. Bis-[2,4-dihydroxy-1,3,5-triazyl - (6) ] - di-  
amino-diphenyl urea disulfonic acid:



11. Bis-[2,4-dihydroxy-1,3,5-triazyl - (6) ] - di-  
amino-diphenyl-thiourea disulfonic acid:



5

10

12. Bis-[2,4-dihydroxy-1,3,5-triazyl - (6) ] - dl-  
aminostilbene disulfonic acid:



15

20

13. Bis-[2-hydroxy-4-phenylamino - 1,3,5 - tri-  
azyl-(6) ]-diaminostilbene disulfonic acid:



25

30

35 14. Bis-[2 - hydroxy - 4 - ortho - chlorophenyl-  
amino-1,3,5-triazyl - (6) ] - diaminostilbene disul-  
fonic acid:



40

45

50 15. Bis-[2-hydroxy - 4 - para - methoxyphenyl-  
amino-1,3,5-triazyl - (6) ] - diaminostilbene disul-  
fonic acid:



55

60

60 16. Bis-[2-aminophenyl-4-aminophenyl -1,3,5-  
triazyl-(6) ]-diaminostilbene disulfonic acid:



65

70

75

17. Bis-[4-(N-ethyl-N-para-sulfobenzyl-para-phenylene diamino) - 2 - hydroxyl - 1,3,5 - triazyl-(6) 1-diaminostilbene disulfonic acid:



18. Bis-[2-hydroxy-4-(5-sulfonaphthylamino) - 1,3,5-triazyl-(6) ]-diaminostilbene disulfonic acid:



19. Bis-[2-hydroxy - 4 - (para - aminophenol - methyl-pyrazolone)-1,3,5-triazyl-(6) ] - diamino-stilbene disulfonic acid:



20. Bis-[2-hydroxy-4-cyclohexylamino - 1,3,5 - triazyl-(6) ]-diaminostilbene disulfonic acid:



21. Bis-[2-dodecylamino-4-sulfo-ethyl-amino-1,3,5-triazyl-(6) ]-diaminostilbene disulfonic acid:



22. 2,6-bis-[2-hydroxy-4-phenoxy-1,3,5-triazyl-(6) ]diaminotoluene sulfonic acid-(4):



23. 2,6-bis-[2-hydroxy-4-(2-mercaptopbenzthiazole-6-amino)-1,3,5-triazyl-(6)]-diaminotoluene sulfonic acid-(4):

The following examples illustrate the invention:

(1) A sheet of regenerated cellulose is bathed



24. 2,6-bis-[2-hydroxy-(4-aminophenylamino)-1,3,5-triazyl-(6)]-diaminotoluene sulfonic acid-(4):

for some minutes with a solution of bis-[2-hydroxy-4-phenylamino-1,3,5-triazyl-(6)]-benzidine disulfonic acid in 100 cc. of water and 2



25. 2-[2,4-dihydroxy-1,3,5-triazyl-(6)-amino]-6-[4-(2,4-dihydroxy-1,3,5-triazyl-(6)-amino)-25 benzamino]-toluene sulfonic acid-(4):

grams of sodium carbonate, then rinsed, treated with a glycerine bath and dried.

(2) For making a sheet of gelatin the gelatin



26. 2,6-bis-(4-[2-hydroxy-4-(4-sulfophenyl-35 amino)-1,3,5-triazyl-(6)-amino]-benzamino)-toluene sulfonic acid-(4):

solution is mixed with the sodium salt of 1,4-bis-[2-hydroxy-4-phenyl-amino-1,3,5-triazyl-(6)-amino-benzene-disulfonic acid-(2,5) in such



50. 27. 1,4-bis-[2-hydroxy-4-quinolylamino-(6)-1,3,5-triazyl-(6)-amino]-benzene disulfonic acid-(2,5):

proportion that the dry sheet contains 0.3 to 1.0 gram of the salt per meter<sup>2</sup>.

(3) For making parchment paper the pulp



28. 5-[2,4-diamino-1,3,5-triazyl-(6)-amino]-7,8-benzoquinoline:

used is mixed with the sodium salt of bis-[2-hydroxy-4-phenylamino-1,3,5-triazyl-(6)-diaminostilbene disulfonic acid in such proportion that 100 kilos of the dry substance contain 0.5 kilo of the agent that protects the goods from damage by light. The pulp is converted into the parchmentized paper in the usual manner.

What we claim is:

1. A process of producing a wrapping material which comprises incorporating in a sheet material permeable to ultraviolet rays a 1,3,5-triazine derivative at most slightly colored.

2. A process of producing a wrapping material which comprises incorporating in a sheet of

70 The sheets may, for example, be saturated with the substance in question in intimate and non-reversible condition by merely immersing it in an aqueous solution of the substance, or the triazine derivative may be incorporated in the sheet in the process of manufacturing the latter.

70



regenerated cellulose the sodium salt of bis-[2-hydroxy-4-phenylamino-1, 3, 5-triazyl-(6)-benzidine disulfonic acid.

3. A process of producing a wrapping material which comprises incorporating in a solution of gelatin the sodium salt of 1, 4-bis-[2-hydroxy-4-phenylamino-1, 3, 5-triazyl-(6)-amino]-benzene-disulfonic acid.
4. A process of producing a wrapping material which comprises incorporating in the pulp used for making parchment paper the sodium salt of bis-[2-hydroxy-4-phenylamino-1, 3, 5-triazyl-(6)-diaminostilbene disulfonic acid.
5. A sheet material permeable to ultra-violet

rays containing a 1, 3, 5-triazine derivative at most slightly colored.

6. A sheet of regenerated cellulose containing the sodium salt of bis-[2-hydroxy-4-phenylamino-1, 3, 5-triazyl-(6)-benzidine disulfonic acid.

7. A sheet of gelatin containing the sodium salt of 1, 4-bis-[2-hydroxy-4-phenylamino-1, 3, 5-triazyl-(6)-amino]-benzene-disulfonic acid.

8. A parchment paper containing the sodium salt of bis-[2-hydroxy-4-phenylamino-1, 3, 5-triazyl-(6)-diaminostilbene disulfonic acid.

JOHN EGGERT.  
BRUNO WENDT.